

## UNITED STATES PATENT OFFICE

2,225,938

## ALLOY WITH ARTIFICIAL RADIO ACTIVITY

Oleg Yadoff, Issy-les-Moulineaux, France

No Drawing. Application December 28, 1936, Serial No. 117,976. In France December 27, 1935

5 Claims. (Cl. 75—140)

(Granted under the provisions of sec. 14, act of March 2, 1927; 357 O. G. 5)

It is known that it was recently discovered that it is possible artificially to produce, under the action of intensive electric fields, alloys capable of emitting rays similar to alpha rays.

5 These emanations are spontaneous, and, because of their low amplitude, their intensity remains constant after a long time.

The object of the present invention is to provide a new alloy of this kind, which is to be called "R alloy," giving a very high activity, and capable, in particular, of acting to a distance through air, fluids, quartz, various dielectrics, etc. The physical structure of the alloy according to the present invention is based upon the general principle of transmutation and the discovery of artificial radio-activity, as above mentioned.

The new alloy according to the present invention is obtained from a charge which chiefly includes aluminium, from 68 to 74%; magnesium, from 4.2 to 8.4%; silicon, from 1.5 to 3.5%; copper, from 5 to 12%; tin, from 4 to 6.5%; lead, from 2.4 to 5%; manganese, from 1.89 to 2%; and mercury, from 0.5 to 1%.

In this alloy the essential elements are aluminium and magnesium. Silicon and tin increase in a substantial manner the activity of the alloy. Copper serves to improve the cohesion and the mechanical properties of the alloy, by forming a kind of binder, but it is not an essential 30 element of the alloy. Lead also serves to improve the radio-active properties and manganese the inductive properties of the alloy. Finally, mercury is intended to purify the alloy.

Preferably, the alloy is of the following composition, which I found to give the best possible results: Aluminium, 73%; magnesium, 6.4%; silicon, 3.2%; copper, 7.5%; tin, 5.1%; lead, 2.4%; manganese, 1.89%; and mercury, not more than 0.5%.

40 In accordance with my invention, this alloy can be prepared as follows:

The alloy can be prepared in any furnace. I first introduce, in the cold state, on the bottom of the furnace, the necessary amount of mercury. I cover the layer of mercury with tin and lead. I place thereabove copper and aluminum in a mixed form, for instance, in the form of an alloy commonly used for automobile pistons. The percentage of aluminum lacking in this alloy for obtaining the desired proportion is introduced in the pure state. Then the furnace is heated until the whole alloy is molten. Mercury evaporates and purifies the composition of the alloy. Then manganese is introduced. About five minutes after complete melting, once mercury has

evaporated, magnesium is introduced into the furnace in a pure state.

The mixture is stirred and the inside of the furnace is subjected to the action of an intensive electric field, for instance, by connecting two circular zones of the furnace to a source of high tension direct current. In order to determine the tension, account is taken of the amount of alloy to be prepared and of the characteristics of the furnace. I may indicate, by way of example, that, for a thickness of ten centimeters of the alloy in the melted state, it is advisable to make use of a source of 3000 volts. The intensive electric field should be applied for ten minutes. Then the tension at the terminals is reduced in 15 a gradual manner in such manner as to pass from full tension to zero tension in a period of time of about two minutes. After this, I operate in substantially the same manner as with ordinary alloys. As a rule, the alloy according to the invention should not be subjected to violent shocks and to sudden variations of temperature.

The present invention is not in any way limited to a special method of producing the alloy, 25 but the above process has proven advantageous and is also set forth in my divisional application, Serial No. 176,643, filed November 26, 1937, now Patent No. 2,175,236.

The alloy which constitutes the chief object 30 of the present invention can be obtained in any suitable manner.

What I claim is:

1. An alloy having artificial radio-activity consisting of from 68 to 74% of aluminium, from 4.2 to 8.4% of magnesium, from 1.5 to 3.5% of silicon, from 5 to 12% of copper, from 4 to 6.5% of tin, from 2.4 to 5% of lead, from 1.89 to 2% of manganese, and not more than 0.5% of mercury. 40

2. An alloy having artificial radio-activity which consists of 73% of aluminium, 6.4% of magnesium, 3.2% of silicon, 7.5% of copper, 5.1% of tin, 2.4% of lead, 1.89% of manganese, and not more than 0.5% of mercury. 45

3. An alloy having artificial radio-activity comprising from 68 to 74 per cent of aluminium, from 4.2 to 8.4 per cent of magnesium, from 1.5 to 3.5 per cent of silicon, from 4 to 6.5 per cent of tin, from 2.4 to 5 per cent of lead, from 1.89 to 2 per cent of manganese, and not more than 0.5 per cent of mercury. 50

4. A charge for the obtainment of an alloy having artificial radio-activity, which consists of from 68 to 74 per cent of aluminium from 4.2 to 8.4 per cent of magnesium, from 1.5 to 3.5 per cent of silicon, from 4 to 6.5 per cent of tin, from 2.4 to 5 per cent of lead, from 1.89 to 2 per cent of manganese, and not more than 0.5 per cent of mercury. 55

to 8.4 per cent of magnesium, from 1.5 to 3.5 per cent of silicon, from 5 to 12 per cent of copper, from 4 to 6.5 per cent of tin, from 2.4 to 5 per cent of lead, from 1.89 to 2 per cent of manganese, and from 0.5 to 1 per cent of mercury.

5. A charge for the manufacture of an alloy having artificial radio-activity, which consists of

73 per cent of aluminium, 6.4 per cent of magnesium, 3.2 per cent of silicon, 7.5 per cent of copper, 5.1 per cent of tin, 2.4 per cent of lead, 1.89 per cent of manganese, and 0.5 per cent of mercury.

OLEG YADOFF. 5